

1,335,176.

M. M. MERRITT,  
ELECTROLYTIC APPARATUS AND METHOD.  
APPLICATION FILED AUG. 2, 1918.

Patented Mar. 30, 1920.

2 SHEETS—SHEET 1.

Fig. 2.



Fig. 1.



Inventor  
Matthew M. Merritt.  
by Emery Booth Janney & Son  
Atty.

M. M. MERRITT.

ELECTROLYTIC APPARATUS AND METHOD.

APPLICATION FILED AUG. 2, 1918.

1,335,176.

Patented Mar. 30, 1920.

2 SHEETS—SHEET 2.

*Fig. 3.*



*Fig. 4.*



*Fig. 5.*



*Inventor:*

*Matthew M. Merritt,*

*by Emery Booth, James V. Varnay  
Atty's.*

# UNITED STATES PATENT OFFICE.

MATTHEW M. MERRITT, OF SOUTH MIDDLETON, MASSACHUSETTS, ASSIGNOR TO  
COPPER PRODUCTS COMPANY, OF BOSTON, MASSACHUSETTS, A CORPORATION  
OF MAINE.

## ELECTROLYTIC APPARATUS AND METHOD.

1,335,176.

Specification of Letters Patent. Patented Mar. 30, 1920.

Application filed August 2, 1918. Serial No. 247,967.

To all whom it may concern:

Be it known that I, MATTHEW M. MERRITT, a citizen of the United States, and a resident of South Middleton, county of Essex, Commonwealth of Massachusetts, have invented an Improvement in Electrolytic Apparatus and Methods, of which the following description, in connection with the accompanying drawings, is a specification, 10 like characters on the drawings representing like parts.

This invention pertains to improvements in electrolytic apparatus and methods, and more particularly, though not exclusively, 15 to improvements in apparatus for and methods of electrolytically depositing copper to protect the tips of aeroplane propellers.

In the drawings:—

Figure 1 is a vertical section, partly in elevation, through a preferred form of apparatus used in connection with my invention;

Fig. 2 is a side elevation thereof, partly in section, on the line 2—2 of Fig. 1;

Fig. 3 is an enlarged view of the end of a propeller shown in Fig. 1;

Fig. 4 is a section on the line 4—4 of Fig. 3; and

Fig. 5 is a view of a complete propeller 30 and its associated apparatus as shown in Fig. 1.

In the drawings I have shown a tank 4 containing electrolyte 5, anodes 6, and having a horizontal rotatable shaft 7 mounted 35 above the tank adapted to carry a plurality of aeroplane propellers 8 mounted thereon, preferably in such relation as to form a helix, the shaft preferably being at such a height above the electrolyte that approximately one-third of a propeller can be immersed in the electrolyte. The shaft 7 is 40 preferably rotated by any suitable mechanism, at such speed that the end portions of each propeller will be immersed approximately two seconds and emersed approximately four seconds.

The end of the propeller which is to be protected by electrolytic deposit is coated with electro-conductive material, preferably 50 bronze powder and amyl-acetate. Adjacent the edge of the portion of the propeller to be coated I preferably provide a narrow band 9 of shellac or other non-conductive material, and adjacent the non-conductive band 55 I preferably provide a "thief" 10 which

may conveniently be formed by a second band of conductive paint. The remainder of the propeller may be protected from the action of the acid in the electrolyte by paraffin or any other suitable acid-resisting substance. About those portions of the propeller which are to be coated, I preferably provide a framework 11 which for convenience may take the form of a box having the ends removed, and which may be secured in 60 place in any suitable way, typified by the wedge-blocks 12 adjacent the hub of the propeller.

By the symmetrical positioning of the propellers about the shaft 7, the amount of 70 electro-conductive surface immersed in the electrolyte is kept substantially constant as the shaft is revolved, thus preventing deleterious variation in the amount of current available for electro-deposit on any given 75 surface at any time. The framework 11 causes the electrolyte to be stirred up in front of the surface on which deposition is to be made, and thereby not only tends to prevent the adhesion of dirt or occluded hydrogen on the cathode by increasing the washing action of the electrolyte, but also tends to minimize that increase of deposit which would otherwise take place on the front edge of the propeller as it revolved. 80 The varnished band 9 gives a clean-cut edge to the electro-deposit, while the "thief" 10 prevents a surplus of deposit on this edge or marginal portion. The "thief" 13 prevents excess deposit and consequent roughness and 85 unevenness of the deposit adjacent the edges of the propeller as distinguished from the edge or marginal portions of the tip which is protected by the "thief" 10.

It will be understood, of course, that the 95 tips of the propellers and the "thieves" 10 and 13 should be connected by wires to the shaft 7, which is connected with any suitable source of current, thereby causing said portions to become cathodes, while the 100 anodes are connected to the opposite pole of the current supply.

Other applications of the fundamental method herein claimed are shown and claimed in my copending applications, Serial No. 247,966, filed August 2, 1918, Serial No. 254,633, filed September 18, 1918, and Serial No. 247,964, filed August 2, 1918.

While I have shown and described apparatus which constitutes a preferred embodiment 110

ment of my invention, and while I have described a preferred way of practising my improved method, it will be understood that major changes in the apparatus and even changes in the method described may be made without departing from the scope of my invention, which is best defined in the following claims.

Claims:

- 10 1. The method of electrolytically depositing metal on segregated surfaces of objects which comprises mounting the objects on a rotatable shaft and rotating the shaft during electro-deposition while a portion only 15 of the surfaces to be deposited upon are immersed in the electrolyte, whereby each surface is alternately immersed and emersed.
- 20 2. The method of electrolytically depositing metal on segregated surfaces of objects which comprises mounting the objects in distributed relation about a rotatable shaft, and rotating the shaft during electro-deposition while a portion only of the surfaces to be deposited upon are immersed in the 25 electrolyte, whereby each surface is alternately immersed and emersed and while the area of immersed cathode surface is maintained substantially constant in area.
- 30 3. The method of depositing metal on a plurality of cathodes which comprises alternately, rapidly and repeatedly immersing and emersing each cathode in the electrolyte.
- 35 4. The method of depositing metal on a plurality of cathodes which comprises alternately, rapidly and repeatedly immersing and emersing each cathode in the electrolyte while maintaining substantially unchanged the aggregate immersed cathode 40 area.

5. The method of depositing metal on a plurality of cathodes which comprises mounting the cathodes in distributed relationship about a rotatable shaft and rotating the shaft during electro-deposition with alternate, rapid and repeated periods of immersion in the electrolyte and emersion therefrom.

6. The method of depositing metal on the tips of aeroplane propellers which comprises mounting the propellers in distributed relationship about a rotatable shaft and rotating the shaft and propellers under partial submergence in an electrolyte while stirring the electrolyte adjacent each propeller tip.

7. The method of depositing metal on the tips of aeroplane propellers which comprises mounting the propellers in distributed relationship about a rotatable shaft and rotating the shaft and propellers under partial submergence in an electrolyte while each propeller tip is preceded by a plow.

8. The method of depositing protecting metal on a propeller tip which comprises coating the end of the tip to be protected with an electrically conductive substance, the edge of the portion to be protected being defined by a band of non-conductive substance, and providing a removable conductive agent adjacent the edge of the portion to be protected, electrolytically depositing metal on the surface to be protected and on the removable conductive agent adjacent the edge thereof, and subsequently removing the removable conductive agent and the metal deposited thereon.

In testimony whereof I have signed my name to this specification.

MATTHEW M. MERRITT.